

Nov. 17, 1942.

U. B. BRAY ET AL

2,302,177

PROCESS FOR SEPARATING WAX FROM OIL

Filed Aug. 22, 1933



## UNITED STATES PATENT OFFICE

2,302,177

## PROCESS FOR SEPARATING WAX FROM OIL

Ulric B. Bray, Palos Verdes, and Claude E. Swift,  
Glendale, Calif., assignors to Union Oil Company of California, Los Angeles, Calif., a corporation of California

Application August 22, 1933, Serial No. 686,254

6 Claims. (Cl. 196—18)

This invention relates to a process for the separation of wax from oil and is a continuation in part of Serial No. 555,018, filed by Ulric B. Bray and Claude E. Swift on August 4, 1931.

The invention relates primarily to a process for the separation of wax from oil by the use of materials which cause wax to be less soluble in oil fractions and which hereinafter will be referred to as wax anti-solvents.

In our prior application, referred to above, we disclosed a process for treating oils to produce lubricating oils which included the steps of diluting the oil with a diluent preferably a liquid normally gaseous hydrocarbon such as liquid propane and then treating the diluted oil with a selective solvent such as liquid sulphur dioxide, acetone, mixtures of acetone and benzol, aniline or methyl formate, for the purpose of splitting the oil into a relatively paraffinic fraction or fraction of high viscosity index and a relatively non-paraffinic fraction or a fraction of low viscosity index. The fraction of relatively high viscosity index containing the propane and a portion of the selective solvent was then chilled to, say, approximately  $-40^{\circ}$  F., preferably by permitting a portion of the propane to vaporize under reduced pressure whereupon wax precipitated from solution. The solution containing the precipitated wax was then filtered to remove the wax from the oil and solvents. The wax-free solution was then chemically treated such as with sulphuric acid and clay after which the remaining propane and liquid sulphur dioxide was vaporized from the treated oil.

In the aforesaid process, we observed that the portion of selective solvent retained in the paraffinic fraction or raffinate phase materially aided in the subsequent separation of the wax from the oil. The present continuation is based upon the foregoing observation and is directed to not only the dewaxing of a raffinate produced by selective solvent extraction but also the dewaxing of other waxy oils which have not previously been subjected to action of selective solvents by commingling the waxy oil with a diluent and a small amount of selective solvents prior to chilling. Furthermore, the selective solvent otherwise known as a wax anti-solvent may not only be added to the oil and diluent prior to chilling but may also be introduced into the diluent oil solution during or upon completion of the chilling operation.

This invention contemplates the use of not only normally gaseous hydrocarbon diluents such as propane, but also such diluents as kerosene, gaso-

line, gas oil, or heavy lubricating oil fractions which are substantially wax-free.

In carrying out the invention the wax containing fraction is dissolved in one of the foregoing diluents. A small quantity of one of the foregoing selective solvents is then added and the mixture is then cooled to a temperature sufficiently low to precipitate the wax. The solution containing the precipitated wax is then filtered, centrifuged or settled to separate the wax from the oil. The de-waxed oil containing the diluent and the wax anti-solvent is then distilled to remove the diluent and anti-solvent from the de-waxed oil.

In carrying out the process as described above the solution of waxy oil diluent and anti-solvent may be chilled by circulating cold brine in indirect heat exchange with the solution to be chilled or by injecting liquid ammonia, liquid sulphur dioxide, liquid carbon dioxide, or other liquid materials which are normally gaseous under ordinary temperatures and pressures into the solution, and allowing these materials to vaporize at a reduced pressure thereby chilling the oil and precipitating the wax.

Another means of chilling consists in adding to the oil normally gaseous hydrocarbons such as liquid propane, liquid ethane, liquid butane, liquid propylene, liquid butylene, and other normally gaseous hydrocarbons along with the wax anti-solvent, and then allowing a portion of the normally gaseous hydrocarbon to vaporize under reduced pressure, thereby chilling the oil and precipitating the wax. The chilled mass is treated in the same manner as described above for the separation of the wax from the oil.

It is therefore an object of this invention to add anti-solvents to waxy oils to aid in the separation of the wax from the oil.

It is a further object of this invention to dilute waxy oils with suitable diluents such as liquid propane, gasoline, kerosene or gas oil, add anti-solvents to this solution of waxy oil and then separate the wax from the oil.

It is a further object of this invention to dilute waxy oils with liquid propane, add anti-solvents selected from the class of sulphur dioxide, aniline, chloraniline, nitrobenzol, dichlorethylether, acetone and benzol or methyl-formate, cool the solution to a temperature sufficiently low to precipitate the wax, and then separate the precipitated wax from the propane solution of oil and anti-solvent.

In carrying out our process a waxy oil is diluted with from 1 to 3 volumes of liquid propane at a

temperature of about 70° F. and under sufficient pressure to maintain the propane in the form of a liquid. The propane solution of oil is then mixed with from 10 to 25% of sulphur dioxide by volume and the mass is then cooled either by vaporizing propane under reduced pressure or by any suitable indirect refrigeration means to a temperature sufficiently low to precipitate the wax. The temperature of the chilled mass will vary. However, in most cases we find that temperatures ranging from 0° F. to minus 20° F. are sufficiently low to precipitate a substantial portion of the wax present in solution. The chilled mass containing precipitated wax is then settled, centrifuged or filtered for the separation of the precipitated wax from the propane solution of oil and sulphur dioxide. The dewaxed oil containing propane and sulphur dioxide is then distilled to separate the propane and sulphur dioxide from the oil.

In some cases more sulphur dioxide or other anti-solvent is added to the oil than remains in the solution at the lowered temperature. In these cases the excess is allowed to settle out and is removed at the end of the chilling step from the chilled mass prior to the separation of the precipitated wax. This is accomplished by allowing the chilled mass to settle for a short time in a quiescent state. As the chilled mass settles in a quiescent state anti-solvents which we have described settle to the bottom of the vessel owing to their relatively high specific gravity. These anti-solvents may then be withdrawn from the bottom of the vessel away from the chilled mass. The chilled mass from which the excess anti-solvent has been removed may then be passed to wax separation means for the separation of the precipitated wax from the propane solution of oil and anti-solvent.

A number of methods may be employed for the addition of the antisolvent to the oil to be dewaxed. For example, the diluent such as liquid propane, kerosene, gasoline or gas oil may be saturated with the antisolvent such as liquid sulphur dioxide at an ordinary temperature. The diluent saturated with antisolvent may then be mixed with a waxy oil. Usually this mixing is carried out at a temperature and under conditions which will render the waxy oil soluble in the diluent containing the antisolvent. This solution is then chilled to a temperature sufficiently low to precipitate the wax. The chilled mass may then be passed to any suitable wax separation means such as the filter press, settling chamber or centrifuge for the separation of the precipitated wax from the chilled mass. The dewaxed oil recovered from the wax separation means may then be distilled in order to separate the diluent and antisolvent from the dewaxed oil.

If desired, the waxy oil may be saturated with an antisolvent such as sulphur dioxide diluted with a suitable diluent as described above, chilled to a temperature sufficiently low to precipitate the wax and the chilled mass may then be filtered, centrifuged or settled to separate the precipitated wax from the mass.

As a further modification of this process a waxy oil may be diluted with a suitable diluent such as liquid propane, gasoline, naphtha, kerosene or gas oil and chilled to a temperature sufficiently low to precipitate the wax. The precipitated wax may then be separated from the mass and then a portion of one of the foregoing anti-solvents may be injected into the chilled mass for 75

the precipitation of a further quantity of wax which may be separated from the diluted oil by any one of the foregoing means.

As a further modification we may inject any one of the antisolvents which we have described continuously during the chilling step or if desired it may be injected after the chilling step and then the precipitated wax may then be separated from the diluents and oil.

It is therefore an object of the present invention to inject antisolvents, selected from the class of aniline, cresylic acid, phenol, chloraniline, sulphur dioxide, nitrobenzol, dichlorethylether, acetone and benzol, and methyl formate into a waxy oil dissolved in a diluent during the chilling step to aid in the separation of the wax from the oil.

It is a further object of the present invention to mix antisolvents with chilled waxy oil and diluent to aid in the separation of the wax from the oil.

It is still a further object of the present invention to dissolve waxy oil in a diluent, chill the mass to a temperature sufficiently low to precipitate wax, separate the precipitated wax from the oil, mix the chilled mass from which the precipitated wax has been separated with an antisolvent such as sulphur dioxide, aniline, phenol, chloraniline, nitrobenzol, dichlorethylether, cresylic acid, acetone and benzol or methyl-formate and separate a further quantity of wax with or without further cooling.

It is still a further object of the present invention to mix a waxy oil with a diluent, chill the diluted waxy oil and then mix the chilled oil with an antisolvent such as sulphur dioxide, phenol, chloraniline, nitrobenzol, dichlorethylether, cresylic acid, methyl-formate, aniline or acetone and benzol to aid in the precipitation of wax from the diluted oil.

It is only necessary to employ sufficient of the foregoing wax antisolvents to saturate the oil at the temperature at which the wax is removed. Any excess of these antisolvents which would tend to produce an oil phase saturated with these wax antisolvents and a phase consisting of antisolvent containing some dissolved oil fractions should be avoided. Where phase separation occurs due to too large an excess of the antisolvent some of the wax fractions may be dissolved in the antisolvent phase containing dissolved oil fractions and thus not be precipitated and removed from the oil during the wax separation step.

Our process may be more easily understood by referring to the figure. Referring more specifically to the figure a waxy oil in tank 1, at a temperature above its congealing point is withdrawn through line 2, valve 3 and line 4 to pump 5 which forces it through line 6 where it meets a stream of diluent coming from tank 8 through valve 9, line 10, pump 11, line 12, mixing coil 13 and line 14. The mixture of waxy oil and diluent in line 6 passes into mixing coil 7 where it is thoroughly agitated. The agitation here in most instances is sufficient to produce a solution of the waxy oil in the diluent. The solution of the waxy oil in the diluent may be facilitated if desired in agitating coil 7 by raising the temperature of the diluent in waxy oil by some means not shown. The solution of a waxy oil in the diluent emerges from agitating coil 7 to line 15 where it is mixed with antisolvent withdrawn from tank 18 through pump 19, line 20, valve 21. The antisolvent passes into line 15 along with the oil and diluent from whence it passes into mixing coil 54 where the

mass is thoroughly mixed. From mixing coil 54 the mass passes into chiller 17 where the temperature of the mass is lowered sufficiently to cause a precipitation of the wax. Where heavy diluents such as naphtha, gasoline, kerosene or gas oil are employed external refrigeration must be supplied to the mixture of diluent oil and antisolvent in chiller 17 in order to attain a temperature sufficiently low to precipitate the wax.

Where a normally gaseous liquefied hydrocarbon such as liquid propane is employed as the diluent in chiller 17 the refrigeration may be obtained by opening valve 28 and allowing a portion of the diluent to vaporize under a reduced pressure. The vaporized diluent being released through valve 28 passes through line 29, pump 30, line 31, pump 46, line 47, condenser 48 and line 49 to receiving tank 50.

In case more antisolvent has been injected into the mass in chiller 17 than remains soluble at the lower temperature, this excess of antisolvent can be settled out by maintaining the mass in chiller 17 in a placid state. The antisolvent collects in the bottom of chiller 17 and is removed by pump 32, line 33, valve 34 and line 35 from the system.

The chilled mass in chiller 17 is then removed through valve 32, line 33, valve 36 and line 37 to wax separation means 38 where the wax is separated and removed to line 39. The dewaxed oil dissolved in solvent is removed through line 40, pump 41 and valve 42 to heater 43. Heat is supplied to the mass in heater 43 by coil 55 through which steam or other heating medium is supplied. The diluent and antisolvent are vaporized in heater 43 and passed through line 44, valve 45, pump 46 and line 47 to condenser 48 where they are condensed. The liquefied diluent and antisolvent pass from condenser 48 through line 49 into collecting chamber 50.

The liquid collected in chamber 50 consists of recovered diluent and antisolvent. This material may be returned to the cycle through line 12. If desired, a further quantity of antisolvent may be injected into the liquid passing from line 53 into line 12 by opening valve 23 and forcing antisolvent through pump 19, line 28, line 22, valve 23 and line 24 into line 12. This mixture of material passing through line 12 from line 53 and antisolvent passing into line 12 from line 24 passes into agitator 13 where the two materials are thoroughly mixed before introduction of these materials into the stream of waxy oil withdrawn from tank 1 into line 6.

The antisolvent in tank 18 may also be employed to saturate the diluent in tank 8 by mixing the fresh diluent withdrawn from tank 8 into line 12 with antisolvent withdrawn from tank 18 through line 24. Fresh diluent in tank 12 and the antisolvent withdrawn through line 24 are mixed in coil 13 and pass through line 14 into line 6 where the diluent containing the antisolvent is mixed with fresh waxy oil withdrawn from tank 1 into line 6.

If desired, the antisolvent may be injected into the oil diluent in cooler 17 during the chilling step. In this case the oil in tank 1 and the diluent in tank 8 are withdrawn as previously described into mixing coil 1 and then pass into chiller 17. As the refrigeration is supplied to the material in chiller 17 by external means or by vaporizing a portion of the diluent, as previously described, antisolvent in tank 18 is introduced into chiller 17 through pump 19, line 20, line 22, valve 25 and line 26.

As a further modification the mixture of oil and diluent in chilling chamber 17 can be completely chilled and then we may add the antisolvent into chilling tank 17 from tank 18 by the method just described.

As we have already stated we may also remove the wax from the oil in steps. In the first step we may not use antisolvent. In this case the oil in tank 1 and the diluent in tank 8 are mixed in coil 1 and are passed into chilling chamber 17. The waxy oil and diluent in chiller 17 are then cooled by external refrigeration or if the diluent is normally gaseous a portion of this material may be vaporized under reduced pressure until a temperature is obtained in chiller 17 at which a portion of the wax is precipitated. The chilled mass in tank 17 is then removed through pump 32, line 33, valve 36, line 37 to wax separation means 38 where the wax is separated from the oil and removed through line 39. The dewaxed oil recovered in line 40 may then be returned to chiller 17 by means not shown in this drawing, and admixed with antisolvent from tank 18 through pump 19, line 20, line 22, valve 25 and line 26.

In some cases it may be necessary to further chill the oil in chiller 17 to obtain any substantial separation of wax, and in some cases the cold material passing from the wax separation means 38 back to chiller 17 is sufficiently cold to obviate the necessity of further refrigeration for the separation of the further quantity of wax provided antisolvents are injected or mixed with this cool material. The cooled mass in chiller 17 is again withdrawn through pump 32, line 33, valve 36 and line 37 to wax separation means 38 where the precipitated wax is separated from the diluent oil and antisolvent.

In some cases it may be found necessary to acid-treat the oil prior to the separation of the wax with diluents and antisolvents. In this case the oil in tank 1 may be an oil which has been previously contacted with sulphuric acid for the separation of materials which hinder the separation of wax from oil.

We have used the term "propane" in this specification to include members of the normally gaseous hydrocarbons such as ethane, propane, butane and mixtures thereof. It is to be understood, however, that other normally gaseous hydrocarbons may be employed in our process to advantage—for example—we may employ liquid ethylene, propylene or butylene or mixtures thereof, or we may employ hydrocarbons which are normally gaseous and which are halogenated—for example—we may employ methyl chloride, ethyl chloride or dichlore-difluor-methane. We may also employ as diluents normally gaseous ethers or normally gaseous halogenated ethers or mixtures thereof.

As a specific example of the method of carrying out our process a Santa Fe Springs distillate having a specific gravity of 32.8° A. P. I. and a pour point of 110° F. was mixed with liquid propane and liquid sulphur dioxide in the following proportions:

|                               | Volume |
|-------------------------------|--------|
| Liquid propane                | 4      |
| Liquid sulphur dioxide        | 1      |
| The Santa Fe Springs waxy oil | 1      |

This mixture was then agitated and cooled by external means at the rate of 1.2° F. per minute until a final temperature of -15° F. was obtained. The chilled mass was then filtered to separate the precipitated wax from the oil, propane and

sulphur dioxide. The filtrate consisting of dewaxed oil, propane and sulphur dioxide was then distilled to remove the propane and sulphur dioxide from the dewaxed oil. The oil dewaxed by the foregoing method had a pour point of 5° F.

It is to be understood that the foregoing examples are merely illustrative of our process and are not to be construed as limiting the invention which we claim.

We claim:

1. A process for the separation of wax from oil comprising mixing said oil with liquid propane, vaporizing liquid propane under reduced pressure to chill the oil, adding a wax antisolvent and separating wax and subsequently separating the separated wax from the oil, remaining liquid propane and wax antisolvent.

2. A process as in claim 1 in which the wax antisolvent is liquid sulphur dioxide.

3. A process as in claim 1 in which the wax 20 antisolvent is added during the chilling step.

4. A process as in claim 1 in which the wax antisolvent is liquid sulphur dioxide and said

liquid sulphur dioxide is added during the chilling step.

5. A process for the separation of wax from oil comprising mixing the oil with a liquid normally gaseous hydrocarbon diluent, chilling said diluted oil to precipitate the wax by vaporizing a portion of the diluent under reduced pressure, adding a wax anti-solvent to the chilled solution containing the precipitated wax and subsequently separating the precipitated wax from the oil, diluent and wax anti-solvent.

15 6. A process for the separation of wax from oil comprising mixing said oil with liquid propane under superatmospheric pressure, chilling the solution of oil and propane to precipitate wax by reducing the pressure to vaporize a portion of the propane, adding liquid sulfur dioxide to the chilled solution containing the precipitated wax and subsequently separating the precipitated wax from the oil, propane and sulfur dioxide.

ULRIC B. BRAY.  
CLAUDE E. SWIFT.